

1

3,429,813

**SYNTHETIC LUBRICANTS CONTAINING PHOSPHOROTHIONATES AND ARYLAMINES**

Francis H. Waight, Eastham, Wirral, and Alexander C. B. MacPhail, Little Sutton, Wirral, England, assignors to Shell Oil Company, New York, N.Y., a corporation of Delaware

No Drawing. Filed Sept. 23, 1964, Ser. No. 398,742  
Claims priority, application Great Britain, Oct. 25, 1963, 10  
42,137/63

U.S. Cl. 252—46.7  
Int. Cl. C10m 3/42

9 Claims

This invention relates to improved synthetic lubricating compositions which are oxidation-stable and which have excellent anti-wear properties. In a preferred aspect the invention relates to improved aircraft turbine lubricants which contain certain esters of phosphorothionic acid in combination with certain amine antioxidants.

Synthetic lubricants have recently gained prominence in the field of lubrication because they are able to meet the more stringent requirements of certain new applications. They have found use in jet aircraft where wide temperature ranges and extreme operating conditions are likely to be encountered. Under these extreme conditions, synthetic oils are often corrosive and undergo thermal and oxidative deterioration resulting in sludge and deposit formation, viscosity change, discoloration and other undesirable changes. Attempts to correct these deficiencies by conventional methods are frequently unsatisfactory because of the extreme nature of the application of the oil. For example, addition of a conventional antioxidant to reduce deterioration may cause increased corrosion, or addition of an antiwear agent might decrease stability. Furthermore, the addition of more than one additive frequently compounds the problem because of incompatibility of the additives. Therefore, although a particular additive might aid oxidation stability, the further addition of a known extreme-pressure agent is likely to detract from the effectiveness of the antioxidant.

It has now been found that certain triaryl esters of phosphorothionic acid are excellent extreme-pressure agents and cooperate with certain known amine antioxidants to markedly improve oxidation resistance of certain synthetic ester lubricants. Accordingly, the invention provides an improved ester-based synthetic lubricant

2

which contains minor amounts of a triaryl ester of phosphorothionic acid as hereinafter defined, an arylamine and/or a thioldiarylamine.

Suitable triaryl esters of phosphorothionic acid contain from six to about fourteen carbon atoms per aryl group. Examples of triaryl esters are triphenyl, tritolyl, tribenzyl, trixylyl, naphthylidiphenyl trianaphthyl, and tri-octyl phenyl phosphorothionates. An especially preferred ester is triphenyl phosphorothionate. The triaryl esters of the invention may be used in concentrations between about 0.5% and 10% by weight, preferably between 2 and 7% by weight based on the final lubricating oil.

Suitable arylamines and thioldiarylamines are described in Mehr et al., U.S. 2,815,327, issued Dec. 3, 1957. Examples of appropriate arylamines are diphenylamine, phenyl- $\alpha$ -naphthylamine, phenyl- $\beta$ -naphthylamine,  $\alpha,\alpha'$ -dimethylamine, methyl phenyl- $\alpha$ -naphthylamine, phenyl- $\beta$ -(butylnaphthyl)amine, and  $\alpha,\beta$ -dinaphthylamine. Diarylamines are preferred. Appropriate thioldiarylamines are phenothiazine, phenylthio- $\alpha$ -naphthylamine,  $\alpha,\alpha'$ -thiodinaphthylamine, and 3,7-dioctyl phenothiazine. In general, for both additive the aryl nuclei are phenyl or naphthyl and may be alkylated with up to four alkyl groups having from one to ten carbon atoms. The amine additives are advantageously used in concentrations of about 0.5% to 5% by weight, preferably 1 to 3% by weight based on the final composition. In an especially preferred aspect of the invention, the triarylphosphorothionate is used in combination with both an arylamine and a thioldiarylamine as defined above.

To illustrate the surprising coaction of the additives of the invention, several representative compositions were formulated and tested in the Rolls Royce Blown Oxidation Test, wherein antioxidant activity is expressed in terms of changes of viscosity and acidity. Referring to Table I, formulations I through VIII were made with one of the specified components of the invention absent. These lubricants were tested against formulations IX through XIV, which were compounded according to the invention. All compositions were tested in the Rolls Royce Oxidation Test. In this test, 250 ml. per minute of air or nitrogen saturated with water vapor are bubbled under controlled conditions through a 50-ml. boil sample at 220° C. for 192 hours. The deterioration of the lubricating oil due to oxidation is then measured in terms of acidity and viscosity changes and benzene insolubles. The results of these tests are reported in Table II.

TABLE I

| Composition of Example (percent wt.)                                             | I     | II    | III   | IV    | V     | VI    | VII   | VIII  | IX    | X     | XI    | XII   | XIII | XIV   |
|----------------------------------------------------------------------------------|-------|-------|-------|-------|-------|-------|-------|-------|-------|-------|-------|-------|------|-------|
| Trimethylol propane tripelargonate                                               | 63.0  | 61.0  | 94.98 | 75.98 | ..... | 60.0  | 58.0  | 58.0  | 58.0  | 91.98 | ..... | 72.98 | 53.0 | ..... |
| Hercolube "A" (C <sub>6</sub> -C <sub>9</sub> acid esters of pentaerythritol)    | 19.5  | 19.5  | ..... | 19.5  | 94.98 | 19.5  | 19.5  | 19.5  | 19.5  | ..... | 91.98 | 19.5  | 19.5 | ..... |
| Hercolube "C" (C <sub>4</sub> -C <sub>7</sub> acid esters of pentaerythritol)    |       |       |       |       |       |       |       |       |       |       |       |       |      | 60.0  |
| Hercolube "F" (C <sub>5</sub> -C <sub>10</sub> acid esters of dipentaerythritol) |       |       |       |       |       |       |       |       |       |       |       |       |      | 36.0  |
| Bis(2,2,4-trimethylpentyl)azetate                                                | 14.48 | 14.48 | ..... |       |       | 14.48 | 14.48 | 14.48 | 14.48 | ..... | 1.5   | 1.5   | 1.5  | 1.5   |
| Phenyl- $\alpha$ -naphthylamine                                                  |       |       |       |       |       |       |       |       |       |       | 1.5   | 1.5   | 1.5  | 1.5   |
| 3,7-dioctyl phenothiazine                                                        |       |       |       |       |       |       |       |       |       |       | 1.5   | 1.5   | 1.5  | 1.5   |
| Triphenyl phosphorothionate                                                      |       | 2.0   | 2.0   | 2.0   | 2.0   |       |       |       |       |       | 2.0   | 2.0   | 2.0  | 2.0   |
| Aroclor 1254 (chlorinated diphenyl)                                              | 3.0   | 3.0   | 3.0   | 3.0   | 3.0   | 3.0   | 3.0   | 3.0   | 3.0   | 3.0   | 3.0   | 3.0   | 3.0  | 1.0   |
| 5-methyl benzotriazole (p.p.m.)                                                  | 25    | 25    | 25    | 25    | 25    | 25    | 25    | 25    | 25    | 25    | 25    | 25    | 25   | 25    |
| Antioxidant "A" <sup>1</sup>                                                     |       |       |       |       |       |       |       |       |       |       | 2.0   |       |      |       |
| Antioxidant "B" <sup>2</sup>                                                     |       |       |       |       |       |       |       |       |       |       | 2.0   |       |      |       |
| D.C. 200/12500 silicone (p.p.m.)                                                 | 5     | 5     | 5     | 5     | 5     | 5     | 5     | 5     | 5     | 5     | 5     | 5     | 5    | 5     |
| Azelai acid                                                                      | 0.02  | 0.02  | 0.02  | 0.02  | 0.02  | 0.02  | 0.02  | 0.02  | 0.02  | 0.02  | 0.02  | 0.02  | 0.02 | 0.0   |

<sup>1</sup>  $\alpha,\alpha',\alpha''$ -(2,4,6-trimethyl-1,3,5-benzenetriyl)tris-(2,6-ditertiarybutyl p-cresol).

<sup>2</sup> 4,4'-(2,3,5,6-tetramethylxylylene)bis-(2,6-ditertiarybutyl p-cresol).

TABLE II

| Composition     | Benzene<br>Insolubles<br>(percent<br>wt.) | Viscosity at 210° F. (cs.) |       |                     | Acid Value<br>(mg.KOH/g.) |       |
|-----------------|-------------------------------------------|----------------------------|-------|---------------------|---------------------------|-------|
|                 |                                           | Initial                    | Final | Percent<br>Increase | Initial                   | Final |
| <u>Example:</u> |                                           |                            |       |                     |                           |       |
| I.....          | Solid                                     | .....                      | ..... | .....               | .....                     | ..... |
| II.....         | Solid                                     | .....                      | ..... | .....               | .....                     | ..... |
| III.....        | Solid                                     | .....                      | ..... | .....               | .....                     | ..... |
| IV.....         | Solid                                     | .....                      | ..... | .....               | .....                     | ..... |
| V.....          | Solid                                     | .....                      | ..... | .....               | .....                     | ..... |
| VI.....         | 0.02                                      | 4.84                       | 19.4  | 305                 | 0.10                      | 6.05  |
|                 | 0.008                                     |                            | 25.1  | 418                 |                           | 6.15  |
| VII.....        | 0.017                                     | 5.08                       | 27.8  | 446                 | 0.10                      | 6.55  |
|                 | 0.008                                     |                            | 18.2  | 258                 |                           | 6.20  |
| VIII.....       | 0.012                                     | 5.04                       | 32.6  | 547                 | 0.10                      | 6.30  |
|                 | 0.008                                     |                            | 59.2  | 1,080               |                           | 6.20  |
| IX.....         | nil                                       | 4.80                       | 11.9  | 148                 | 0.10                      | 4.90  |
|                 | nil                                       |                            | 12.0  | 150                 |                           | 4.60  |
| X.....          | 0.003                                     | 5.02                       | 13.5  | 169                 | 0.10                      | 4.00  |
|                 | 0.02                                      |                            | 13.6  | 171                 |                           | 3.10  |
| XI.....         | 0.005                                     | 4.90                       | 12.2  | 149                 | 0.10                      | 4.45  |
|                 | 0.005                                     |                            | 12.4  | 153                 |                           | 3.35  |
| XII.....        | 0.004                                     | 5.00                       | 13.6  | 172                 | 0.10                      | 4.80  |
|                 | 0.02                                      |                            | 13.2  | 164                 |                           | 4.70  |
| XIII.....       | 0.006                                     | 5.04                       | 11.7  | 132                 | 0.10                      | 3.75  |
|                 | 0.01                                      |                            | 12.1  | 140                 |                           | 3.65  |
| XIV.....        | 0.05                                      | 5.47                       | 9.43  | 72.5                | 0.20                      | 4.60  |
|                 | 0.01                                      |                            | 10.13 | 85.2                |                           | 3.60  |

Table II shows that the use of a triaryl ester of phosphorothionic acid imparts essentially no antioxidant activity when used alone in a synthetic ester lubricating oil (Examples I-V). Examples IX-XIV evidence the enhanced antioxidant activity imparted by the triaryl esters to the known amine antioxidants. This increase is shown by the reduction in benzene insolubles, viscosity increase, and acid value resulting from the addition of the phosphorothionate to the amine-containing oil. The increase in antioxidant activity is indeed even greater than that attributable to other well known antioxidants used in combination with an aryl amine and a thiadiazylamine (Examples VII and VIII).

The phosphorothionic acid esters can be prepared in any manner known to the art. For example, thiophosphoryl chloride can be prepared from sulfur and phosphorous trichloride and can subsequently be reacted with the appropriate phenol in the presence of a Friedel-Crafts catalyst such as aluminum chloride. Alternately, phosphorus trichloride can be added at temperatures of from about 50 to 150° C. to a mixture of elemental sulfur with an appropriate phenol to yield the desired ester in a one-step process.

Although the additive combination of the invention is generally applicable to both synthetic and mineral lubricating oils, it is particularly desirable for use in synthetic oils. Synthetic ester lubricants are especially preferred.

Preferred synthetic lubricant base stocks are esters of alcohols having 1 to 20, especially 4 to 12, carbon atoms and aliphatic carboxylic acids having from 3 to 20, especially 4 to 12, carbon atoms. The ester base may be a simple ester (reaction product of a monohydroxy alcohol and a monocarboxylic acid), a polyester (reaction product of an alcohol and an acid, one of which has more than one functional group, or a complex ester (reaction product of a polyfunctional acid with more than one alcohol, or of a polyfunctional alcohol with more than one acid). Also, excellent synthetic lubricants may be

40 formulated from mixtures of esters, such as major proportions of complex esters and minor amounts of diesters.

Monohydric alcohols suitable for making ester base stocks include methyl, butyl, isoctyl, dodecyl and octadecyl alcohols. "Oxo" alcohols prepared by the reaction of olefins with carbon monoxide and hydrogen are suitable. Neo alcohols, i.e., alcohols having no hydrogens on the beta carbon atom are preferred. Examples of such alcohols are 2,2,4-trimethylpentanol-1 and 2,2-dimethyl propanol.

50 Polyalcohols used for the production of base oil esters preferably contain 1 to 12 carbons. Examples, of di-alcohols are 2-ethyl-1,3-hexanediol, 2-propyl-3,3-heptanediol, 2-butyl-1,3-butanediol, 2,4-dimesityl-1,3-butanediol, and polypropylene glycols having molecular weights from about 100 to 300. Alcohols having three, four, five or more hydroxyl groups per molecule are also suitable 55 and are preferred; examples of these polyols are pentaerythritol, dipentaerythritol, and trimethylolpropane. Mixtures of alcohols may also be used.

Suitable carboxylic acids for making the ester base oils include mono- and dibasic aliphatic carboxylic acids. Examples of appropriate acids are butyric, valeric, sebacic, azelaic, suberic, caproic, adipic, ethyl suberic, glutaric, pentadecanedicarboxylic, thiodiglycolic, propionic, caprylic, pimelic, and mixtures thereof. Preferred acids are sebacic, azelaic, glutaric, adipic, and their mixtures.

60 Examples of suitable ester base oils are ethyl palmitate, ethyl laurate, butyl stearate, di(2-ethylhexyl) sebacate, di(2-ethylhexyl) azelate, ethyl glycol dilaurate, di(2-ethylhexyl) phthalate, di(1,3-methylbutyl) adipate, di(1-ethylpropyl) azelate, diisopropoxylate, dicyclohexyl 70 sebacate, glycerol tri-n-heptoate, di(undecyl) azelate, and tetraethylene glycol di(2-ethylene caproate), and mixtures thereof. A preferred mixture of esters consists of about 50 to 80% wt. bis(2,2,4-trimethylpentyl) azelate and 20 to 50% wt. 1,1,1-trimethylpropyl triheptanoate.

Especially preferred esters for use as base stocks in the present invention are esters of monocarboxylic acids having three to twelve carbons and polyalcohols such as pentaerythritol, dipentaerythritol, and trimethylolpropane. Examples of these esters are pentaerythrityl tetrabutyrate, pentaerythrityl tetracaproate, pentaerythrityl dibutyrate-dicaproate, pentaerythrityl butyratecaproate divalerate, pentaerythrityl butyrate trivalerate, pentaerythrityl tributylatecaproate, mixed C<sub>4</sub>-10 saturated fatty acid esters of pentaerythritol, dipentaerythrityl hexavalerate, dipentaerythrityl hexaheptoate, dipentaerythrityl tributylatecaproate, dipentaerythrityl trivalerate trinonylate, dipentaerythrityl mixed hexaesters of C<sub>4</sub>-10 fatty acids and trimethylolpropane heptylate. Pentaerythritol esters of mixtures of C<sub>4</sub>-C<sub>12</sub> acids are excellent base oils, and are commercially available from Hercules Chemical Company.

Ester oils may be prepared by simple reaction of the alcoholic and acidic reactants in proportions suitable for producing the desired product; preparation preferably takes place in a solvent such as an aromatic hydrocarbon, and in the presence of a catalyst, such as HC1, HF, HBr, H<sub>2</sub>SO<sub>4</sub>, H<sub>3</sub>PO<sub>4</sub>, SOC<sub>1</sub><sub>2</sub>, BF<sub>3</sub>, etc. Preparation of suitable esters is described in Eichemeyer, U.S. 3,038,859, issued June 12, 1962, and Young, U. S. 3,121,109, issued Feb. 11, 1964.

The lubricants of the invention may contain any other additives known to be beneficial in synthetic lubricants, such as additional extreme-pressure agents, thickeners, anti-lacquering agents, antifoam agents, dyes, and anti-corrosion agents.

We claim as our invention:

1. A lubricant composition comprising a major amount of a synthetic ester base, 0.5 to 10% by weight of a triaryl ester of phosphorothionic acid having 6 to 14 carbons per aryl group, and 0.5 to 5% by weight of at least one member of the group consisting of diarylamines containing one to two rings per aryl group substituted with zero to four alkyl groups having one to ten carbon atoms and thioldiarylamines having a thiazine nucleus, said thioldiarylamines being substituted with zero to four alkyl groups having from one to ten carbon atoms.

2. A composition of claim 1 wherein the triaryl ester of phosphorothionic acid is triphenyl phosphorothionate.

3. A lubricant composition comprising a major amount of a synthetic ester base, 0.5% to 10% by weight of a triaryl ester of phosphorothionic acid having from six to fourteen carbons per aryl group, 0.5% to 5% by weight

of a diarylamine having one to two rings per aryl group substituted with zero to four alkyl groups having from one to ten carbon atoms, and 0.5% to 5% by weight of a thioldiarylamine having a thiazine nucleus and having one to two rings per aryl group substituted with zero to four alkyl groups having from one to ten carbon atoms.

4. The lubricant of claim 3 wherein the triaryl ester of phosphorothionic acid is triphenyl phosphorothionate.

5. The lubricant of claim 4 wherein the diarylamine is phenyl- $\alpha$ -naphthylamine.

6. The lubricant of claim 4 wherein the thioldiarylamine is selected from the group consisting of phenothiazine and 3,7-diethyl phenothiazine.

7. A lubricant composition comprising a major amount of a synthetic ester base, 0.5 to 10% by weight of triphenyl phosphorothionate, 0.5 to 5% by weight of phenyl- $\alpha$ -naphthylamine, and 0.5 to 5% by weight of 3,7-diethyl phenothiazine.

8. A lubricant composition comprising a major amount of a synthetic ester base, 0.5 to 10% by weight of triphenyl phosphorothionate, 0.5 to 5% by weight of phenyl- $\alpha$ -naphthylamine, and 0.5 to 5% by weight of phenothiazine.

9. A lubricant composition consisting essentially of a major amount of a synthetic ester base lubricant, a minor stabilizing amount of a triaryl ester of phosphorothionic acid having 6 to 14 carbon atoms per aryl group and a minor amount of a diarylamine selected from the group consisting of diarylamines having one to two rings per aryl group, ring alkylated derivatives thereof, thioldiarylamines having a thiazine nucleus, and ring-alkylated derivatives thereof, said amine being present in an amount sufficient to enhance the oxidative stability imparted by said organophosphorus compound.

#### References Cited

##### UNITED STATES PATENTS

|           |         |                 |       |          |
|-----------|---------|-----------------|-------|----------|
| 2,242,260 | 5/1941  | Prutton         | ----- | 252—46.6 |
| 3,100,748 | 5/1963  | Richards et al. | ----- | 252—46.6 |
| 3,218,256 | 11/1965 | Edwards et al.  | ----- | 252—47   |

DANIEL E. WYMAN, Primary Examiner.

W. H. CANNON, Assistant Examiner.

U.S. Cl. X.R.

252—46.6, 49.9